# EUROPEAN PATENT SPECIFICATION

(11) **EP 1 050 054 B1**
(45) Date of publication and mention of the grant of the patent: **07.03.2007**
(21) Application number: 99901767.6
(22) Date of filing: 21.01.1999
(51) Int. Cl.: H01C 7/02

(54) **POLYMER COMPOSITION**
POLYMERZUSAMMENSETZUNG
COMPOSITION POLYMERE

(30) Priority: 23.01.1998 WO PCT/GB98/00206; 28.03.1998 GB 9806623; 30.06.1998 GB 9814130
(43) Date of publication of application: 08.11.2000
(73) Proprietor: Peratech Limited, Durham DL1 4PJ (GB)
(72) Inventor: LUSSEY, David, Richmond, North Yorkshire DL10 7QL (GB); KING, Andrew, Brian, Thirsk, North Yorkshire YO7 4RW (GB); LUSSEY, Christopher, John, Richmond, North Yorkshire DL10 7QL (GB)
(74) Representative: Naylor, Matthew John
(86) International application number: PCT/GB1999/000205
(87) International publication number: WO 1999/038173

(56) References cited:
- DE-A- 4 315 382
- GB-A- 2 054 277
- US-A- 5 106 540
- US-A- 5 591 382

## Description

### TECHNICAL FIELD

This invention relates to a polymer composition including a finely divided electrical conductor, particularly comprising such a composition in an advantageous physical form.

### BACKGROUND ART

The use of such a composition has been proposed for devices for controlling or switching electric current, to avoid or limit disadvantages such as the generation of transients and sparks which are associated with the actuation of conventional mechanical switches.

In particular, co-pending application PCT/GB98/00206 dated 23rd January 1998 and subsequently published under serial number WO98/33193, discloses such a composition and switches based on it. That application discloses for the first time a granular composition containing polymer and conductive filler. The present application relates to a polymer composition in that form and to further developments thereof.

DE-A-4315382, to which corresponds US-A-5589222, discloses hydrophobic flowable granules comprising hydrophilic inorganic powder and 0.03 to 15% w/w of hydrophobic polyorganosiloxan and a process of producing them by mixing the powder in a granulator with an aqueous emulsion of the polyorganosiloxan and drying the resulting product at elevated temperature. Among the powders listed are metals and alloys. The granules are, however, for use in enamelling; there is no disclosure that they might form part of an electrical circuit or, further, that they could be electrically insulating when quiescent but conducting when subject to mechanical stress or electrostatic field.

US-A- 5106540 discloses a composition with a matrix polymer and a particulate conductive filler distributed therein, such as carbon black. A composite filler is produced by melt-extruding and then comminuting the extrudate. The composite filler is then blended with polymer to form a resistive component.

### SUMMARY OF THE INVENTION

According to the present invention there are provided granules comprising at least one substantially non-conductive polymer and at least one electrically conductive filler selected from powder-form metallic elements and alloys, electrically conductive oxides of said elements and alloys, and mixtures thereof, and said electrically conductive filler has a dendritic, filamentous or spiked structure whereby said granules are electrically insulating when quiescent but conductive when subjected to mechanical stress or electrostatic charge.

The invention further provides a process defined by the features of claim 5, a composite defined by the features of claim 7, a composite structure defined by the features of claim 8, a use defined by the features of claim 10 and an electromagnetic shield defined by the features of claim 11.

The granules are typically in the size range up to 1mm, especially 0.04 to 0.2mm. Thus the smaller granules behave as powders. The ranges are based on measuring the greater diameter of the granules if not regularly spherical. To suit user's requirements, the granules may be for example in an approximate Poisson size distribution, or sieved to a skewed distribution or a narrow spread (for example, largest granules no greater than 2 x smallest) or classified so that small granules fill the spaces between larger granules.

Within the granules the conductor: polymer volumetric ratio (tapped bulk: voidless solid) is suitably at least 3:1. For the ratio of conductive medium to polymer small changes will be required to account for differences in relative surface tensions of types and grades of polymer and the various surface energies of the different conductive oxides and other solids present. Changes of this ratio have an effect on the piezo-charge properties, the overall resistance range, the recovery hysteresis and the pressure sensitivity of the granules.

In general the conductive material can be one or more metals, other conductive or semiconductive elements and oxides or intrinsically conductive or semiconductive organic or inorganic polymers. Thus it is suitably selected from powdered forms of the metallic elements or their electrically conductive alloys or reduced oxides either on their own or together. More specifically it is one or more of titanium, tantalum, zirconium, vanadium, niobium, hafnium, aluminium, silicon, tin, chromium, molybdenum, tungsten, lead, manganese, beryllium, iron, cobalt, nickel, platinum, palladium, osmium, iridium, rhenium, technetium, rhodium, ruthenium, gold, silver, cadmium, copper, zinc, germanium, arsenic, antimony, bismuth, boron, scandium and metals of the lanthanide and actinide series and, if appropriate, at least one electroconductive agent. The conducting filler can be the basic element in the unoxidised state; or can be a layer on a carrier core of powder, grains, fibres or other shaped forms. The oxides can be mixtures comprising sintered powders of an oxycompound. The alloy may be for example titanium diboride.

The micro-structure of the conductor particles is of substantial importance. Thus dendritic, filamentous, and spiked forms of the conductive materials have been shown to be capable of producing particularly sensitive granules when coated with a polymer such as silicone. Generally the conductor particles are rough-surfaced with smaller and spikier powders producing more sensitive granules. Preferably the particles comprise metal having at least one of these characteristics:
(i) spiky and/or dendritic surface texture;
(ii) filamentary structure, with a three-dimensional chain-like network of spiky beads, the chains being on average 2.5 - 3.5 microns in cross-section and possibly more than 15 - 20 microns in length.

Generally these characteristics are present in the conductor particles before mixing with polymer, and mixing is controlled to substantially preserve them.

As described further below, preferred conductor particles comprise carbonyl-derived metallic nickel. Other examples include dendritic copper.

The polymer constituent of the granules can be chosen from a wide range of materials, the only limitation being that the polymer or a precursor thereof should be available in a form sufficiently mobile to permit incorporation of conductor particles. In an extreme case it can be a fully or partly cured resin, such as a formaldehyde condensate, epoxy resin, maleimide resin or 3-dimensional olefin resin. Polymers having flexibility, such as linear thermoplasts, are of more general application. Very suitably the polymer constituent is an elastomer. Since elastomers are preferred in certain composites including the granules, they will be described further below.

The invention provides a method of making the granules by mixing conductor particles with liquid-form polymer in granule-forming conditions. The liquid-form polymer may be, for example, a precursor subject to polymerization or to cross-linking during the granule-forming step or later. Liquid-form means sufficiently flowable to undergo mixing with the conductor particles. The polymer may be very viscous. A liquid may be present to modify the viscosity of the polymer as an aid to mixing. It may be added, for example, by pre-mixing with the polymer or with the conductor powder. The liquid should of course be chemically inert with respect to the conductor and polymer. Preferably it is volatile, that is, has an atmospheric pressure boiling point under 120°C, to assist removal during and after mixing. Hydrocarbons, such as petroleum distillates, are very suitable. Before or during mixing there may be added a hydrophobising agent. This is believed to act by displacing adsorbed water from the surfaces of the components of the mix, for example the conductor particles, solid additives such as those described below, especially fumed silica, and possibly of newly exposed polymer and newly formed granules. The agent may also act as a lubricant limiting friction at mixer surfaces. Since it can act by formation of very thin, even unimolecular layers, the quantity to be used is very small, for example 10 - 1000 ppm w/w of the mix. Examples of the agent are liquid hydrocarbons carrying groups favouring chemisorption on metals, and fluorocarbons.

The granules are made by coating conductive particles with a layer of polymer in a controlled mixing regime that imparts only sufficient force to the components of the mix to achieve the coating process and avoids additional force which has been found to have a degrading effect on the electrical properties of the final polymer composition. The relationship between filler, binder, mixing energy, time, rate of shear, temperature and pressure determine the particle size-distribution and electro-mechanical properties of the resulting granule. It appears likely that the conductor particles act as nuclei for granule formation. Such mixing is preferably at a low level of shear, so that the conductor particles remain structurally intact. Suitably a dish-granulator, blunger, coaxial cylinder mixer (rotary ablation) can be used. In the granule-forming step it appears that the total shear can be of the same order as in the production of bulk composition but applied at greater intensity for a shorter time.

Granule formation is preferably accompanied by some cross-linking of the polymer. The polymer formulation is chosen and the conditions of mixing are controlled so that breakage of the mixture into granules is synchronized with cross-linkage of the polymer sufficient for a non-sticky state. This is especially convenient using RTV silicone. The process may if desired be controlled to produce a precursor of the granules in which the polymer may be subjected to further cross-linking to develop elastomerism. Use of HTV silicone affords more scope in making such precursors. The silicone very suitably is one subject to high shrinkage for example by 10 - 20% on cross-linking. This makes possible a relatively high conductor to polymer volume ratio in granules without an inconveniently high ratio at the start of mixing.

If the silicone content of the mix is increased, sensitivity is decreased and agglomeration increases. If high silicone content is required, silicone may be applied to previously made granules of lower silicone content. In rotary ablation the clearance setting of the pestle against the mortar, and the pressure applied to the pestle, are mechanically adjusted to achieve the required conditions. This pressure affects the time taken to achieve the granulated state and is important to the coating thickness, the eventual size of the granule and the amount of agglomeration between individual granules. Too much pressure produces destructive shear forces.

The resulting granules can be comminuted to provide a desired range. They can be screened to separate the different sized agglomerations if required. Different sized granules show different sensitivities; granule sizes can be separated and remixed in different proportions to alter the final sensitivity of the granule composite. It has also been found possible to combine different conductive materials, conductive, semi-conductive or non-conductive powders, prior to the granule-forming agglomeration/coating process to obtain the required conduction or other electrical and mechanical properties in the final granule form.

The invention provides also a composite comprising the granules. Generally the granules can be used by containing them in a device which limits peripheral movement but allows the input of an electrical or mechanical pressure in order to activate it. They may be mixed with or coated onto other bulk or foamed polymers to form solid, semi-flexible or flexible composite structures. For one type of structure, the granules can be extruded or pressed into sheet, pellet or fibre form or can be cast into moulds. In the course of the shaping process they can be milled or cryogenically powdered. Energy imparted during mixing and moulding the polymer composition in the uncured state may, however, affect the physical and electrical performance of the composite.

For a second type of composite, the granules may be associated with a containing means. This may be a fibre or sheet, for example of polymer fibre film, plate or cloth and may carry granules on one or both faces. The polymer sheet may already contain or carry conductor particles as described for example in Example 7 of the co-pending application. The sheet may comprise or carry an adhesive for the granules.

In another method of forming such a composite, precursor granules (as specified above) can be pressed into the surface or surfaces of the un-cross-linked carrier polymer and permanently bonded to the carrier polymer when it is cross-linked. This produces a pressure sensitive or EM screening layer on the carrier polymer.

For a third type of composite the granules are associated with a three-dimensional matrix. The matrix may be electrically non-conducting, but could be composed, for example, of polymer having conductor particles dispersed in it , such as described in the co-pending application or in prior-published documents. Several variants of this type are possible, for example:
(i) added granules individually conducting or non-conducting or mixed;
(ii) matrix material differing in degree of cross-linking from granule polymer;
(iii) matrix material may enter spaces between granules or may be just a containment bag.

In a particular example of the third type, in which the polymer composition may be in bulk form as described in the co-pending application or, preferably, introduced in granule form as follows:
in a composite structure for generation, detection and relay of electrical signals internal connectivity is provided in the form of an integrated electrically conductive member for example a layer such as metal film or sheet especially continuous metallised cloth, typically polyester based. The cloth increases the tactile sensitivity (increase in resistance drop versus mass loading) of the conductive polymer composition by providing a hard fibre anvil for elastomeric distortion and provides an electron bridge between zones of low resistance within the composite. The polymer composition can be bonded to or formed on the conductive member.

Whereas the composite may be a simple device for switching on when deformed, more complicated electrical circuits may be built into the layer, for example, of the metallised cloth structure. The metal coated fabric is typically manufactured by application of metal by vapour deposition, sputtering or similar means to a woven polyester cloth.

Electrical circuits, analogous to those etched onto a conventional printed circuit board, may be created by masking and etching the pre-metallised cloth or preferably by masking the target cloth at the point of metallisation.

In the latter example the metal coating will only be deposited where the mask allows and by this process a conductive circuit layout can be produced.

Composites incorporating the circuit cloth show true flexibility, are solid state and may be made extremely sensitive to touch or other operating forces. They may be used for digital and analogue switching and control, may incorporate PTC load control or heat production capability and have the capacity to carry substantial electric currents.

Whichever type of composite is in view, a particularly useful one comprises the granules and includes means for the input of electrical and/or mechanical deformation to activate it. Thus the sheet or matrix would comprise ohmic conductor (s) connecting the granule assembly electrically.

The granules can also be used as a component of other conductive and electromagnetic shielding materials either alone or in combination with Other powders or granules or other non-conductive, semiconductive or conductive materials.

Granule-coated surfaces can be particularly sensitive to applied pressure, increasing in pressure sensitivity with increasing surface loading. Granules on their own and granule-coated surfaces can show a drop in electrical resistance of more than 10¹² ohms with an applied force within the range 0.01 - 6 N/cm².

Whichever type of composite is being made, it is preferred to have a hydrophobising agent , as above described, present when an assembly of the granules is being set up.

Composites containing the granules as a film or heterogeneous mixture with other polymers and materials tend to show greater repeatability, sensitivity and linearity of resistance change than can be obtained with bulk pressure sensitive polymer compositions as in the co-pending application. Like the bulk composition, the granules return to a quiescent resistance state when the operating force is removed.

For the granules and/or the matrix (especially if conducting), very suitably the polymer constituent is an elastomer, especially having the general properties:
i) low surface energy typically in the range 15 - 50 dyne/cm but especially 22 - 30 dyne/cm;
ii) a surface energy of wetting for hardened elastomer higher than its uncured liquid;
iii) a low energy of rotation (close to zero) giving extreme flexibility;
iv) excellent pressure sensitive tack both to the filler particles and electrical contacts to which the composite may be attached - that is, possess a high ratio of viscous to elastic properties at time spans comparable to bonding times (fraction of a second);
v) high on the triboelectric series as a positive charge carrier (conversely, will not carry negative charge on its surface);
vi) chemically inert, fire extinguishing and effective as a barrier to oxygen and air ingress.

Silicone elastomer rubbers are typically but not exclusively based on polydimethylsiloxane, polysilamine and allied silicone backbone polymers, with leaving groups, cross-linkers and cure systems based on:

| **Leaving Group** | **Cross Linker** | **Cure System** |
|---|---|---|
| HOC (O) CH₃ | CH₃Si[OC(O)CH₃]₃ | ACETIC ACID |
| HOCH₃ | CH₃ Si (OCH₃)₃ | ALCOHOL |
| HONC (CH₃) (C₂H₅) | CH₃Si [ONC (CH₃) C₂H₅]₃ | OXIME |
| CH₃C (O) CH₃ | CH₃Si [CH₂C (O) CH₃]₃ | ACETONE |
| HN (CH₃) C (O) C₆H₅ | CH₃Si [N (CH₃) C (O) C₆H₅] | ₃ BENZAMIDE |

meet all the above mentioned property criteria. The elastomer can be mixtures comprising cured elastomers selected from the group comprising one, two or more component silicones, one, two or more component polygermanes and polyphosphazines and at least one silicone agent. In such polymer mixtures, the silicone component exceeds other polymer components.

Other additives are included with the silicone for the purpose of modifying the physical and/or electrical properties of the uncured or cured polymer composition. Such additives can include at least one property modifier from the group comprising: alkyl and hydroxyalkycellulose, carboxymethylcellulose, hydroxyethylcellulose, hydroxypropylcellulose, polyacrylamide, polyethylene glycol, poly (ethylene oxide), I polyvinyl alcohol, polyvinylpyrrolidone, starch and its modifications, calcium carbonate, fumed silica, silica gel and silicone analogues and at least one silica analogue or silicone analogue modifier. Fumed silica is an example of a modifier as commonly used in elastomer technology. For this invention, in proportions of between 0.01 - 20% by weight of the final polymer composition, it acts as a recovery-enhancing filler, that is, it increases the resilience of the polymer composition to accelerate the return of the composition to its quiescent state after any applied force is released. A preferred example of a silicone system is manufactured from high strength room temperature cured fumed silica loaded (RTV) silicone polymer. Another example uses high temperature cured HTV silicone filled with fumed silica to provide interstitial structure, useful strength, pressure tack and life, cross-linked at an elevated temperature in the presence of a peroxide or other catalyst, that may typically but not exclusively be 2,4 dichloro dibenzoyl peroxide. Such HTV products may be stored for prolonged periods in the uncured state prior to processing into sheet, rod, foam, fibre, press moulded or other forms.

Another usable class of elastomer is the natural or synthetic hydrocarbon rubbers. Especially for matrix material, such rubber may be introduced in latex form.

The resulting composites may display a piezo-charge affect and will change their inherent electrical resistance in response to both pressure and strain forces. Working resistance is around the range 10¹² to 10⁻¹ ohms and the composites have excellent current carrying capability; typically a 2mm thick sample of the composite on a heat-sink can control AC or DC currents of 3A/cm². The initial application of pressure or force to a sample of the high-resistance composite results in the generation of an electrostatic charge; increasing the pressure or force decreases the electrical resistance of the composite. The composites can be flexible and can reassert themselves when the force or pressure is removed. As this occurs the electrical resistance will increase towards a quiescent value and a pronounced electrostatic charge will develop. The electrostatic effect can provide digital switching indications or provide a voltage source. The electrical resistance change can provide an analogue of the applied pressure or force. Alternatively, the resistance range can be used to provide digital switching especially but not essentially at its upper and lower limits. Sensitive versions of composite which are close to conduction, can be changed into a fully conducting state by applying an electrostatic charge, typically that generated by a piezoelectric spark generator and greater than 0.5kV.

The composite may consist of the granules held within a matrix. Within the granules the conductive particles are of such a size distribution as to provide for a close packed structure with interstitial particle infilling. Voids present in the bulk conductor powder become infilled with elastomer during mixing and conductor particles become set in close proximity during curing. In order to achieve this structural arrangement the elastomer will have a low surface energy relative to the powder phase and uncured liquid surface energy less than cured elastomer surface energy. Such polymer compositions will include silicones, polygermanes and polyphosphazines. In the stressed state the distortion takes place such that the average entrapped inter-particle distance decreases. For metal particles this corresponds to an increase in electrical conductivity, for other types of particle other effects may be generated (change in ferromagnetism, piezoelectricity, ionic conduction, etc.).

For metal filled compositions over the transition from unstressed to stressed state, bulk conductivity will change from that of the elastomer to that of the entrapped conductor particles. At a certain level of distortion the number of particle-to-particle open-circuit tracks results in a conductivity tending towards that of the bulk metal resistivity. Since this effect is ultimately related to distortion of the bulk composite, and since the bulk material is highly elastomeric and therefore energy absorbing, low 'metallic' conductivity may only be achieved for thin sections (less than 2mm in lateral dimension) of the composite material or upon application of high external stress or strain or torque. Upon removal of external force the material reverts to its original structure whereby entrapped particles are held apart within an elastic insulating network.

Surprisingly, the assembly of granules is capable of carrying significant electrical current. Up to 30 amps continuous load has been carried by a 2 x 2cm conductor to date when in a compressed state. This unique property may be explained by the fact that in the compressed state conduction occurs principally through the metal bridges described above. So for the purpose of explaining conduction the materials are best described in terms of a heterogeneous mixture in which the insulative encapsulant dominates electrical property in the quiescent state; and tending towards that of the conductor bridges (having a local resistivity tending to that of the conductor typically 1 - 1000 microhm-cm), in the compressed state (typically having a bulk resistivity greater than 1 milliohm-cm). Electron conduction is further confined to the conductor filler by the inability of the encapsulant to hold negative 'electron' charge (typically the encapsulant is the optimal positive triboelectric charge carrier). For fixed composition the statistical chance of bridge formation is directly related to composite thickness. Thus both the sensitivity to distortion and current carrying capability increase with reduction in thickness with the thinnest films limited by the filler size distribution. For the mixtures described below the filler size distribution will typically limit thickness to >10 - 40 microns.

By incorporation of zirconium particles (or other ionic conducting materials) into a silicone elastomer, within and/or between granules, the composite may be made to conduct both electrons and, in the presence of gaseous oxygen, oxygen ions. By control of bulk material stress (for example by the incorporation of static or externally resonated 'stress grids' into the bulk composition) conduction of electrons and oxygen may be made to occur in different planes or different parts of the bulk structure. Such properties may be of particular interest in the design of fuel cell systems. It has also been found that internal ohmic heating may affect the internal structure of the composite. So for example in compositions encompassing nickel as conductive filler, RTV silicone encapsulant and fumed silica skeletal modifier, it is found that the differential expansion of the encapsulant relative to the conductor is of such proportion (typically, the encapsulant expands fourteen times faster than the conductor) that upon passage of high current, sufficient to create ohmic heating, differential expansion alters the stress/strain versus resistance transition. This effect may be induced at low differential temperatures (typically less than 100°C). This effect (which induces a positive temperature coefficient of resistance (PTC) in the composite phase) may be conveniently employed for the purpose of regulating current flow. Onset of PTC may be regulated by increasing or decreasing mechanical pressure on the polymer composition. Alternatively, for composites that have a low electrical resistance (typically <100 ohms) in the quiescent state, ohmic heating switches by virtue of the PTC effect between conducting and insulating states in a composition that is under little or no compressive force. This effect allows these polymer compositions to be used as switches or fuses which switch sharply to a high resistance state in response to excess current and which, because of their elastomeric nature, will return to a conductive state without the removal of power when the current flow returns to a set value. This PTC effect can also be used in self-regulating heating elements where heat levels can be set by applying mechanical pressure to keep the polymer composition close to its PTC point at the required temperature. The polymer composition will maintain a relatively steady temperature by cycling in and out of the PTC phase. The composition has wide temperature tolerance and good thermal conductivity.

A nickel powder used in the invention was INCO Type 287 which has the following properties: beads are on average 2.5 - 3.5 microns in cross-section; chains may be more than 15 - 20 microns in length. It is a filamentary powder with a three-dimensional chain-like network of spiky beads having a high surface area. Consistent with this structure its bulk density is 0.75 - 0.95 g/cm².

The sizes of the particles are substantially all under 100 microns, preferably at least 75% w/w being in the range 4.7 to 53 microns.

In particular example, the particle size distribution (in microns and by weight) is as follows (in rounded % figures): 2.4 - 3%, 3.4 - 5%, 4.7 - 7%, 6.7 - 10%, 9.4 - 11%, 13.5 - 12%, 19 - 15%, 26.5 - 15%, 37.5 - 11%, 53 - 8%, 75 - 4%, 107 - below 1%.

Other nickel powders also made by the carbonyl process usable in the invention are:
- Type 123:: bulk density 1.6 - 2.6 g/cm²; equiaxial shape, spiked irregular surface;
- Type 210 :: 96% under 100 microns. apparent density less than 0.5g/cm²; filamentary powder of average particle size 0.5 - 1.0 microns;
- Type 255:: bulk density 0.5 - 0.65g/cm²; filamentary powder with 3 - dimensional chain-like network of very spiky beads cross-section 2 - 3 microns; chain length 20 - 25 microns; 91% under 100 microns.

The above data are quoted from the trade literature of the INCO Speciality Powder products London GB - SW1H 0XB.

Generally the conductor particles have a bulk density less than one third of their solid density.

The composition may be usefully employed in association with the anode or cathode construction of an electrochemical cell based on lithium, manganese, nickel, cobalt, zinc, mercury, silver or other battery chemistry including organic chemistry. Either or both the electrodes may be exchanged or coated with the polymer composition to give the following advantages:
(i) the cell could incorporate its own integral pressure switch which, for example, could be operated by the pressure normally used to hold the cell in place in the battery compartment. By this means, self-discharge or short circuiting of the cell could be reduced or eliminated whilst the cell was in an unstressed storage state;
(ii) the integral pressure switch could simplify circuit design and permit new applications by eliminating the need for external switches;
(iii) as the polymer composition can be manufactured without metal, it is possible to construct a wholly plastic electrochemical cell.

Pressure sensitive polymer composition can also be used without direct involvement in the cell chemistry by positioning the composition on external casings or non-reacting surfaces of electrodes. Switching of the polymer composition could be initiated by externally applied mechanical pressure such as finger pressure or spring pressure from within a battery compartment. This could form a switch for controlling external circuits including battery check circuits.

Other applications of the composition include:

Mechanical Transducers, both relative and absolute, for measuring pressure, load, displacement, torque, elongation, mass and volume change, acceleration, flow, vibration and other mechanically induced changes. Current Flow Transducers.
Electric and Magnetic Field Transducers.
Thermal Energy Transducers.
Magnetostrictive Devices. Magnetoresistive Devices.
Magnetic Resonance Devices.
Detecting and Quantifying Localized Movement of Body Parts and Organs.
Detection and Generation of Sound Waves.
Relay Contacts and Junctions.
Electrical Conductors and Inductors for Microcomponents. Temperature Control.
Screening of Electric and Magnetic Waves.
Current and Voltage Protection Devices.
Switching.

### Power Control.

### BRIEF DESCRIPTION OF THE DRAWING

Figs.1(a) and 1(b) are graphs showing the variation/dependence of resistance with applied pressure for the granules according to the invention.

### DETAILED DESCRIPTION OF THE INVENTION

### EXAMPLE 1

Granules were prepared from:

| | |
|---|---|
| INCO nickel powder 287 | 28g |
| ALFAS Industries RTV silicone type 2000 | 4g |

[This weight ratio corresponds approximately to a nickel : polymer volume ratio of 70 : 1 based on the tapped bulk volume of the nickel and the voidless volume of the silicone]

The silicone as a soft lump was placed in the bottom of a RETSCH RM100 motorized mixer having a steel mortar and a porcelain rotary pestle. The nickel powder was placed around the lump of silicone. The pestle was lowered under hand control with an approximate 1mm clearance from the wall of the mortar. This machine subjects the mixture to rotary ablation. In about 5 minutes the silicone coated the nickel particles and in so doing became resolved into granules having the following size distribution % w/w in microns:

| Size fraction | %w/w |
|---|---|
| + 152 | 32 |
| 152 to 75 | 33 |
| 75 to 45 | 32 |
| - 45 | less than 3 |

Completion of granule formation was evident from a change in the colour and texture of the mixture. During mixing, the cross-linking reaction of the silicone produced the odour of acetic acid; this could be continued further if desired, but mixing was shopped when or soon after the granules had been formed, to avoid risking shear damage to the nickel particles in the granules.

The granules are non-conductive in the quiescent state but are very sensitive to applied pressure.

### EXAMPLE 2

The procedure of Example 1 was repeated using:

| | |
|---|---|
| ALFAS Industries RTV silicone type 1000 | 6g |
| INCO nickel powder 287 | 30g |

corresponding to a nickel: polymer ingredient volume ratio of approximately 50 : 1. Although the ratio is lower than in Example 1, the characteristic shrinkage on cross-linking of the grade of silicone used, resulted in granules electrically conductive without applied pressure. The shrinkage seems to be a product of the loss of volatile components at cross-linking. ALFAS 1000 contains 12% of volatile substances. (ALFAS 2000 contains 4% of volatile substances).

Such granules are for example of especial value in conductive adhesives, EM screening and PTC devices.

### EXAMPLE 3

Example of a conductor based on the granules:
a test piece conductor was made by loading a sample of the granules prepared in Example 1 into a test cell consisting of a washer of silicone rubber sponge 12mm in diameter, 3mm thick and with a hole 6mm in diameter, resting on an electrically conductive surface as lower electrode. A conductive plate was placed on top of the washer to form an upper electrode. The electrodes were connected via a constant-current 10 volt supply and a 20M ohm high-impedance buffer amplifier to a Picoscope ADC 100 signal processor and recording device. To allow measured amounts of force to be applied to the test cell, it was placed on the platen of a load testing device, namely a Lloyd Instruments LRX fitted with a 100N maximum force resolver. Slowly increasing pressure was applied to the cell and its resistance was recorded and represented graphically by the signal processor. Runs were carried out at two levels of current:
   Fig.1(a) 10mA, (resistance in ohms x10²), and
   Fig. 1(b) 1 microA, (resistance in ohms x10⁶).

The figures, in which load and resistance are plotted against time, show that as pressure increased the resistance of the granules in the cell decreased and caused a change in the potential difference (PD) voltage across the cell.

### EXAMPLE 4

Demonstration of non-ohmic conduction:
the test cell of Example 3 was compressed with a static loading of approximately 3N, a current of 10 microAmps was passed through the test cell and its resistance, calculated from the potential difference (PD) across the cell, was 100K Ohms. Keeping the voltage and applied pressure constant, the current was increased to 100 microAmps. The measured PD now showed the resistance of the cell to have dropped to 50K ohms.

### EXAMPLE 5

Example 1 was repeated with the difference that the starting materials were:

| | |
|---|---|
| INCO nickel powder 287 | 30g |
| Dow Corning HTV silicone (20 Shore) | 6g |
| under 50°C petroleum (lighter fuel) | 2g |
| 2,4-dichloro-dibenzoyl peroxide | 200mg |

Granules were formed at the end of about 5 minutes, during which the petroleum evaporated off and sufficient (but incomplete) cross-linking of the silicone took place. The granules were fully cross-linken by heating at 120°C for 20 minutes and were then tested as described in Examples 3 and 4.

### EXAMPLE 6

Example 1 was repeated with the difference that, before being added to the mixer, the nickel powder was sprayed with an aerosol of the hydrophobising agent WD40 (RTM). The granules were tested as in Examples 3 and 4 and found to be substantially more sensitive than those prepared without the WD40.

### EXAMPLE 7

Granules made as in Example 1 were formulated as follows:

| | |
|---|---|
| 45 - 75 micron fraction | 0.225g |
| 75 - 152 micron fraction | 0.225g |
| 25% in water hexadecyl-trimethylammonium chloride | 0.1g |
| Natural rubber latex (60% w/w) | 0.12g |
| Water | 0.15g |

The ingredients, excluding latex, were mixed to form a paste. The latex was added and further mixed to form a gel. The gel was split in two and applied through a stencil onto:
(a) copper coated polyimide printed circuit, and
(b) nickel coated polyester cloth printed circuit.

The resulting structure was dried at 80 - 90°C for 30 minutes, or until dry.

A similar result was obtained using dodecylbenzenesulphonate in place of the hexadecyl-trimethylammonium chloride.

## Claims

1. Granules comprising at least one substantially non-conductive polymer and at least one electrically conductive filler selected from powder-form metallic elements and alloys, electrically conductive oxides of said elements and alloys, and mixtures thereof **characterised in that** said electrically conductive filler has a dendritic, filamentous or spiked structure, whereby said granules are electrically insulating when quiescent but conductive when subjected to mechanical stress or electrostatic charge.

2. Granules according to claim 1 in which the conductive filler : polymer volumetric ratio is at least 3:1.

3. Granules according to claim 1 or claim 2 in which the filler comprises carbonyl-derived metallic nickel.

4. Granules according to any one of the preceding claims in which the polymer is a silicone rubber and contains a recovery-enhancing filler.

5. A process for the production of granules comprising mixing particles of at least one electrically conductive filler selected from powder-form metallic elements and alloys, electrically conductive oxides of said elements and alloys, and mixtures thereof and having a dendritic, filamentous or spiked structure, with a substantially non-conductive liquid-form polymer in granule-forming conditions at a low level of shear whereby the conductive filler particles remain substantially structurally intact.

6. A process according to claim 5 in which such mixing and granule formation is accompanied by cross-linking of the polymer, and the polymer formulation is chosen and the conditions of mixing are controlled so that breakage of the mixture into granules is synchronized with cross-linkage of the polymer sufficient for a non-sticky state.

7. A composite comprising granules according to any one of claims 1 to 4 in association with a polymeric matrix material.

8. A composite structure for generation, detection and relay of electrical signals wherein internal conductivity is provided in the form of an integrated electrically conductive member, the structure including a composite according to claim 7.

9. A composite according to claim 7 for regulating current flow, said composite being a PTC composite and having containing means and having means for input of electrical and/or mechanical deformation to activate the PTC effect of the composite.

10. Use of a composite according to claim 9 for regulating current flow.

11. An electromagnetic shield comprising granules according to any one of claims 1 to 4 or a composite according to claim 7.

## Patentansprüche

1. Körnchen, die zumindest ein im Wesentlichen nicht leitendes Polymer und zumindest einen elektrisch leitenden Füllstoff umfassen, wobei der elektrisch leitende Füllstoff aus pulverförmigen Metallelementen und Legierungen, elektrisch leitenden Oxiden der Elemente und Legierungen und Gemischen davon ausgewählt ist, **dadurch gekennzeichnet, dass** der elektrisch leitende Füllstoff eine verzweigte, faserartige oder zackenartige Struktur aufweist, wodurch die Körnchen im Ruhezustand elektrisch isolierend, jedoch bei mechanischer Beanspruchung oder elektrostatischer Ladung leitend sind.

2. Körnchen nach Anspruch 1, worin das Volumenverhältnis zwischen leitendem Füllstoff und Polymer zumindest 3:1 ist.

3. Körnchen nach Anspruch 1 oder 2, worin der Füllstoff über Carbonyl hergestelltes metallisches Nickel umfasst.

4. Körnchen nach einem der vorangegangenen Ansprüche, worin das Polymer ein Siliconkautschuk ist und einen Erholungs-verbessernden Füllstoff enthält.

5. Verfahren zur Herstellung von Körnchen, umfassend das Vermischen von Teilchen zumindest eines elektrisch leitenden Füllstoffs, der aus pulverförmigen Metallelementen und Legierungen, elektrisch leitenden Oxiden der Elemente und Legierungen und Gemischen davon ausgewählt ist und eine verzweigte, faserartige oder zackenartige Struktur aufweist, mit einem im Wesentlichen nicht leitenden Polymer in Flüssigform unter Körnchenbildungsbedingungen bei geringer Scherkraft, wodurch die leitenden Füllstoffteilchen im Wesentlichen strukturell intakt bleibt.

6. Verfahren nach Anspruch 5, worin ein solches Vermischen und eine solche Körnchenbildung von der Vernetzung des Polymers begleitet ist und die Polymerbildung so gewählt ist und die Mischbedingungen so reguliert sind, dass das Aufbrechen des Gemischs in Körnchen mit dem Vernetzen des Polymers abgestimmt ist, um einen ausreichend nicht-klebrigen Zustand zu erhalten.

7. Verbundmaterial, das Körnchen nach einem der Ansprüche 1 bis 4 zusammen mit einem Polymermatrixmaterial umfasst.

8. Verbundstruktur zur Bildung, Detektion und Weiterleitung elektrischer Signale, worin die innere Leitfähigkeit in Form eines integrierten elektrisch leitenden Elements bereitgestellt ist, wobei die Struktur ein Verbundmaterial nach Anspruch 7 umfasst.

9. Verbundmaterial nach Anspruch 7 zur Regulierung des Stromflusses, wobei das Verbundmaterial ein PTC-Verbundmaterial ist und Aufnahmemittel sowie Mittel zur Eingabe elektrischer und/oder mechanischer Verformung zur Aktivierung der PTC-Wirkung des Verbundmaterials aufweist.

10. Verwendung eines Verbundmaterials gemäß Anspruch 9 zur Regulierung des Stromflusses.

11. Elektromagnetische Abschirmung, die Körnchen nach einem der Ansprüche 1 bis 4 oder ein Verbundmaterial nach Anspruch 7 umfasst.

## Revendications

1. Granules comprenant au moins un polymère sensiblement non conducteur et au moins une charge électriquement conductrice sélectionnée parmi des éléments métalliques sous forme de poudre et des alliages, des oxydes électriquement conducteurs desdits éléments et alliages, et leurs mélanges **caractérisés en ce que** ladite charge électriquement conductrice a une structure dendritique filamentaire ou en épi, ce par quoi lesdits granules sont électriquement isolants quand ils sont au repos, mais conducteurs quand ils sont soumis à un effort mécanique ou une charge électrique statique.

2. Granules selon la revendication 1 dans lequel le rapport volumétrique charge conductrice: polymère est d'au moins 3:1.

3. Granules selon la revendication 1 ou la revendication 2 dans lesquels la charge comprend du nickel métallique dérivé de carbonyle.

4. Granules selon l'une quelconque des revendications précédentes dans lesquels le polymère est un caoutchouc de silicone et il contient une charge améliorant la récupération.

5. Procédé de production de granules comprenant le mélange de particules d'au moins une charge électriquement conductrice sélectionnée parmi des éléments et alliages métalliques en forme de poudre, des oxydes électriquement conducteurs desdits éléments et alliages, et leurs mélanges et ayant une structure dendritique, filamentaire ou en épi, avec un polymère sous forme liquide qui est sensiblement non conducteur dans des conditions de formation de granules à un faible niveau de cisaillement, ce par quoi les particules de charge conductrice restent sensiblement structurellement intactes.

6. Procédé selon la revendication 5 dans lequel un tel mélange et une telle formation de granules est accompagné par une réticulation du polymère, et la formulation du polymère est choisie et les conditions de mélange sont contrôlées de façon qu'une rupture du mélange en granules soit synchronisée avec une réticulation du polymère suffisante pour un état non-collant.

7. Composite comprenant des granules selon l'une quelconque des revendications 1 à 4 en association avec un matériau de matrice polymérique:

8. Structure composite pour la production, la détection, et le relais de signaux électriques où une conductivité interne est obtenue sous la forme d'un élément électriquement conducteur intégré, la structure comprenant un composite selon la revendication 7.

9. Composite selon la revendication 7 pour réguler l'écoulement de courant, ledit composite étant un composite de PTC et ayant des moyens le contenant, et ayant des moyens pour l'entrée d'une déformation électrique et/ou mécanique pour activer l'effet PTC du composite.

10. Utilisation d'un composite selon la revendication 9 pour réguler l'écoulement de courant.

11. Blindage électromagnétique comprenant des granules selon l'une quelconque des revendications 1 à 4 ou un composite selon la revendication 7.
